

Dec. 7, 1943.

H. F. HOWARD ET AL

2,336,177

HEATING PROCESS

Filed July 11, 1941

2 Sheets-Sheet 1



Inventors  
Harold F. Howard &  
William Richards

By  
Baldwin, Spencer & Fleet  
Attorneys

Dec. 7, 1943.

H. F. HOWARD ET AL

2,336,177

HEATING PROCESS

Filed July 11, 1941

2 Sheets-Sheet 2



Fig. 2.



Fig. 3

Inventors  
Harold F. Howard &  
William Richards

By  
12 Blackmar, Spencer & Clark  
Attorneys

## UNITED STATES PATENT OFFICE

2,336,177

## HEATING PROCESS

Harold F. Howard and William Richards, Flint,  
Mich., assignors to General Motors Corpora-  
tion, Detroit, Mich., a corporation of Delaware

Application July 11, 1941, Serial No. 401,888

1 Claims. (Cl. 219—3).

The present invention relates to the method of manufacture of valves and the like consisting of heating one end of a rod to forging heat and then forging the end into the shape of the head of the valve. In order to confine the heating to one portion of the rod, avoid the formation of scale, and secure other advantages later discussed, heating is done by means of high frequency electricity. The present invention has to do with improvements in the method of heating disclosed in our copending application filed October 7, 1938, now U. S. Patent 2,275,763 granted March 10, 1942.

In early work with this method use was made of rotary generators producing comparatively low frequency current, i. e., on the order of three kilocycles and it was found that small, restricted portions of the rods could not be heated to forging temperature in the desired short period of time. Nor were satisfactory results obtained by employing substantially higher frequencies, e. g., on the order of five kilocycles.

Experimentation with higher frequencies soon revealed that even doubling or trebling the frequency failed to give the rapid ferrous-stock heating desired because of the fact that when a temperature in the neighborhood of 1200° F. was attained no further heating took place for the reason that 1200° F. is in the neighborhood of the Curie point for the steel employed, that is, the critical temperature above which the magnetic permeability is very small. Because of the abrupt falling off of magnetic permeability it appeared that the frequencies required to heat the metal above its Curie point would be so high as to be impracticable to attain because of the cost and inefficiency of the electrical equipment employed.

After much research and experiment, applicants discovered that rods of  $\frac{3}{8}$ " alloy steel such as is employed for internal combustion engine valves might be terminally or otherwise resistively locally heated to forging temperature (2000° F.) in 7.5 seconds by subjecting the rod portion to be forged to the magnetic field induced in an air-core winding energized by an undamped current of ultra-high frequency, i. e., above the 10,000 cycle-per-second limit conceded by authorities to be the practical upper limit for rotary alternators of the Alexanderson and Goldschmidt types employed for heating on a production scale. As fully brought out in our copending application, now Patent No. 2,275,763, the time available for heating such rod stock must be practically momentary to preclude the

formation of a substantial scale coating on such alloy steels which is destructive to even the best and most expensive forging dies. More than this, by such substantially instantaneous local heating of a restricted section of the rod stock, followed by prompt forging, the economies of efficient heating as well as simplified support for the stock during forging are realized. In accordance with this invention, only that portion of the rod which is to be forged is heated to a degree of plasticity such that warpage or other deformation may occur. Still further, since with such instantaneous heating material conduction of heat throughout the valve blank is precluded prior to forging, the operator is able manually to transfer the blank from furnace to the forging press and thence to the bin or conveyor by bare hand without suffering the slightest burn or discomfort.

In applying their discovery to the heating of alloy steel rod stock for fabricating valves and the like, applicants found that undamped currents having a frequency of from 125,000 to 140,000 cycles per second effected uniform through heating of alloy-steel rod stock having a diameter of  $\frac{3}{8}$  of an inch in a matter of seconds, a forging temperature of 2000° F. being realized in approximately 7 to 8 seconds of time. For a disclosure of a preferred embodiment of their invention, reference is made to the accompanying drawings, wherein:

Figure 1 illustrates diagrammatically the electrical equipment employed.

Figure 2 is a longitudinal section through the heating coil assembly.

Figure 3 is a fragmentary view taken on line 3—3 of Figure 2.

Figure 4 is a fragmentary view taken on line 4—4 of Figure 2.

In the case of the valve rod heating operation referred to, a suitable source of electrical energy such as a 3 phase, 4800 volt, 60 cycle power line is indicated in Figure 1 as supplying energy to a step-up transformer preferably having a 1:3 ratio of transformation supplying a suitable rectifier, preferably of the type employing two element tubes, which in turn supplies rectified current at approximately 8500 volts to a suitable vacuum tube oscillator unit as indicated. A separate 220 volt, 3 phase, 60 cycle supply is used for the tube filaments and for auxiliary apparatus such as the pump supplying cooling water to the oscillator and coils H through a suitable high frequency transformer T, the secondary of which supplies current preferably through a coaxial cable indicated at C to a plurality of heating coils

H arranged in series. The coaxial cable consists of coaxial tubular conductors separated by ceramic insulators in accordance with conventional construction. Suitable controls are provided for the rectifier and oscillator and the usual switches, relays and timers, fuses, circuit-breakers and the like may be employed as desired. Water cooling is provided as usual for the oscillator and coils H. Provision may be made for adjustment of the oscillator circuit to produce the frequency desired. The oscillator and the oscillator output circuit must be very carefully shielded to prevent interference with radio receiving and broadcasting for the oscillator itself constitutes a powerful radio sending station, lacking only a suitable antenna and modulation to render it usable for broadcasting. Coaxial cable is non-radiating which eliminates the necessity of shielding.

As shown in Figures 2 to 4, coils H are mounted in housing 12 which is preferably made of insulating material and is provided with a copper lining 14 for shielding. As is best shown in Figures 3 and 4 coaxial cable C is connected to the coils H through suitable fittings 16. The fittings and coils are formed of hollow tubing so that cooling water may be circulated through them through input connection 18 and output connection 20 from a suitable pump, not shown. Coils H are surrounded by jackets 22 of insulating material and are lined with sleeves 24 likewise of insulating material, the coils and linings being mounted on insulating supports 25 and positioned at the opposite ends by insulating bushings 26. From the latter tubular insulators 28 extend to the outside of the box to permit ready insertion to the parts to be heated. Suitable means may be provided to limit the extent of inward movement of the valve rod stock into the heating coils. We have indicated diagrammatically a support 30 carrying supporting pins 32. It is to be understood that the parts last described, together with the insulating sleeves, liners and supports are constructed of material having not only good electrical insulating properties but also high resistance to heat. For this purpose we may employ insulating material made of various refractory oxides or mixtures of oxides.

In heating the rod it is but necessary to insert it in one of the coils H, as indicated at R in Figure 2, and in seven or eight seconds with apparatus of the capacity next specified the rod end will be heated to the desired forging temperature.

It will be noted that the work circuit is illustrated as a tuned circuit, condenser 10 being of sufficient capacity to effect tuning when a valve rod is being heated in each of the coils H. When there are no valve rods in the coils the circuit is completely detuned so that very little current flows in the load circuit and the energy consumed in the heating equipment is likewise very small.

In heating  $\frac{3}{8}$ " diameter valve rod stock to approximately 2000° F. in approximately eight seconds, it has been found desirable to use fre-

quencies of from 125,000 to 140,000 cycles, preferably the latter. A power input of approximately 125 kv.-a. is required. The heating coil current is preferably on the order of 220 amperes.

5 It will be understood that the figures given constitute but one specific example of the application of our invention.

In general, ultra-high frequency current may be employed according to our invention for the heating of any and all metals to forging or welding temperatures or, if desired, by use of higher frequencies to accomplish melting. The method is just as applicable to non-ferrous or non-magnetic materials as it is to ferro-magnetic materials for the major portion of the heating is accomplished by resistance to the flow of eddy currents rather than by hysteresis effect.

This method of heating possesses many advantages:

20 The cost per heating unit actually used in heating the stock is relatively low. This is because the equipment does not consume any substantial amount of energy except when the metal is being heated in the coil and, since the equipment contains no moving parts, the maintenance cost is negligible as compared with the maintenance cost of furnaces, resistance welders or other conventional forms of heating apparatus. It has previously been pointed out that the process gives an improved product free from scale and thereby lengthens die life. No complicated temperature controlling apparatus is required as it is but necessary to properly adjust the generating unit to give the desired heat output in the 35 time cycle required. Because of these and other advantages it is expected that a multitude of uses of ultra-high frequency heating will develop in manufacture.

We claim:

40 A 10-second forging method for solid ferrous rods such as internal combustion engine valve blanks of  $\frac{3}{8}$ " diameter which are subject to die-destructive rapid scale formation at forging temperatures of 2000° F., comprising: placing the 45 portion of the solid ferrous rod which is to be forged inside an air-core winding having magnetic field definition closely corresponding to the rod portion to be forged, energizing said winding from a source of undamped oscillating current having a frequency on the order of 125,000 cycles per second and a value of approximately 100 kv.-a. per ounce of said rod portion to be forged, maintaining said rod portion within the field produced by said thus-energized winding for a period of approximately one-million cycles within a time-duration of less than 10 seconds, and immediately withdrawing said ferrous rod from said winding and subjecting the thus-treated portion thereof to the action of forging dies before appreciable scale formation can occur.

HAROLD F. HOWARD.  
WILLIAM RICHARDS.